



US005389204A

## United States Patent [19]

Ampulski

[11] Patent Number: 5,389,204

[45] Date of Patent: Feb. 14, 1995

[54] PROCESS FOR APPLYING A THIN FILM CONTAINING LOW LEVELS OF A FUNCTIONAL-POLYSILOXANE AND A MINERAL OIL TO TISSUE PAPER

[75] Inventor: Robert S. Ampulski, Fairfield, Ohio

[73] Assignee: The Procter & Gamble Company, Cincinnati, Ohio

[21] Appl. No.: 212,436

[22] Filed: Mar. 10, 1994

[51] Int. Cl.<sup>6</sup> ..... D21H 21/22

[52] U.S. Cl. ..... 162/135; 162/112; 162/158; 162/164.3; 162/164.4; 162/164.6; 162/173; 162/184; 162/206; 162/207; 162/175

[58] Field of Search ..... 162/158, 173, 164.4, 162/206, 207, 184, 164.3, 164.6, 112, 175, 427/391

[56] References Cited

U.S. PATENT DOCUMENTS

|           |         |                    |           |
|-----------|---------|--------------------|-----------|
| 2,826,551 | 3/1958  | Geen               | 252/89    |
| 3,301,746 | 1/1967  | Sanford et al.     | 162/113   |
| 3,438,807 | 4/1969  | Pikula             | 117/154   |
| 3,755,071 | 8/1973  | Bey et al.         | 162/184   |
| 3,814,096 | 6/1974  | Weiss et al.       | 128/260   |
| 3,818,533 | 6/1974  | Scheuer            | 15/104.93 |
| 3,964,500 | 6/1976  | Drakoff            | 132/7     |
| 3,967,030 | 6/1976  | Johnson et al.     | 428/266   |
| 3,974,025 | 8/1976  | Ayers              | 162/113   |
| 3,994,771 | 11/1976 | Morgan, Jr. et al. | 162/113   |
| 4,028,172 | 6/1977  | Mazzarella         | 162/164 R |
| 4,112,167 | 9/1978  | Dake et al.        | 428/154   |
| 4,191,609 | 3/1980  | Trokhman           | 162/113   |
| 4,300,981 | 11/1981 | Carstens           | 162/109   |
| 4,355,021 | 10/1982 | Mahl et al.        | 424/28    |
| 4,376,149 | 3/1983  | Martin             | 428/266   |
| 4,395,454 | 7/1983  | Baldwin            | 428/290   |
| 4,447,294 | 5/1984  | Osborn, III        | 162/158   |
| 4,469,840 | 9/1984  | Alberts et al.     | 524/500   |
| 4,481,243 | 11/1984 | Allen              | 428/154   |
| 4,513,051 | 4/1985  | Lavash             | 428/212   |
| 4,637,859 | 1/1987  | Trokhman           | 162/109   |
| 4,795,530 | 1/1989  | Soerens et al.     | 162/11    |

|           |         |                 |         |
|-----------|---------|-----------------|---------|
| 4,940,513 | 7/1990  | Spendel         | 162/112 |
| 4,950,545 | 8/1990  | Walter et al.   | 428/446 |
| 4,959,125 | 9/1990  | Spendel         | 162/158 |
| 5,059,282 | 10/1991 | Ampulski et al. | 162/111 |
| 5,164,046 | 11/1992 | Ampulski et al. | 162/111 |
| 5,215,626 | 6/1993  | Ampulski et al. | 162/112 |
| 5,227,242 | 7/1993  | Walter et al.   | 428/446 |
| 5,246,545 | 9/1993  | Ampulski et al. | 162/112 |
| 5,246,546 | 9/1993  | Ampulski        | 162/112 |

FOREIGN PATENT DOCUMENTS

|         |        |                    |           |
|---------|--------|--------------------|-----------|
| 899223  | 5/1972 | Canada             | 154/72    |
| 0144658 | 6/1985 | European Pat. Off. | D21H 1/02 |
| 3420940 | 1/1985 | Germany            | .         |

Primary Examiner—Peter Chin

Attorney, Agent, or Firm—Bart S. Hersko; E. Kelly Linman; Jacobus C. Rasser

[57] ABSTRACT

Disclosed is a process for making soft tissue paper which includes providing a dry tissue web and then applying a sufficient amount of a functional-polysiloxane softener compound to the dry web. The softener application process includes the steps of mixing a functional-polysiloxane compound with a suitable nonvolatile diluent, such as a mineral oil, forming an emulsion containing the functional-polysiloxane compound and nonvolatile diluent using a volatile solvent, such as water, and surfactant emulsifier, applying the emulsion to a heated transfer surface, evaporating the volatile solvent from the emulsion to form a film, and then contacting the dry tissue web with the heated transfer surface. Preferably, the tissue web is dried to a moisture level below its equilibrium moisture content before application of the functional-polysiloxane material. The process may further include the steps of applying an effective amount of a surfactant material to enhance softness and/or wettability control; and/or an effective amount of a binder material such as starch, for linting control, and/or to contribute tensile strength to the tissue paper.

23 Claims, 1 Drawing Sheet





Fig. 1

**PROCESS FOR APPLYING A THIN FILM  
CONTAINING LOW LEVELS OF A  
FUNCTIONAL-POLYSILOXANE AND A  
MINERAL OIL TO TISSUE PAPER**

**TECHNICAL FIELD**

This invention relates, in general, to a process for preparing tissue paper; and more specifically, to a process for preparing tissue paper having a soft, silky, flannel-like tactile feel; and enhanced tactile perceivable bulk, and physiological surface smoothness.

**BACKGROUND OF THE INVENTION**

Soft tissue paper is generally preferred for disposable paper towels, and facial and toilet tissues. However, known methods and means for enhancing softness of tissue paper generally adversely affect tensile strength. Tissue paper product design is, therefore, generally, an exercise in balancing softness against tensile strength. Both mechanical and chemical means have been introduced in the pursuit of making soft tissue paper: tissue paper which is perceived by users, through their tactile sense, to be soft. Such tactile perceivable softness may be characterized by, but not limited to, friction, flexibility, and smoothness; and subjective descriptors such as feeling like silk or flannel. The present invention pertains to a process for improving the tactile perceivable softness of tissue paper—in particular high bulk, creped tissue paper—through the incorporation of chemical additives: in particular, polysiloxane materials which impart a silky or flannel-like feel to the tissue paper without rendering it greasy or oily to the tactile sense of users of products comprising such tissue paper. Additionally, surfactant material may be added to further enhance softness and/or surface smoothness and/or to at least partially offset any reduction in wettability caused by the polysiloxane; and binder material such as starch may be added to at least partially offset reductions in strength and or increasing in linting proclivity that results from the polysiloxane and, if used, the surfactant additive.

Representative high bulk, creped tissue papers which are quite soft by contemporary standards, and which are susceptible to softness enhancement through the present invention are disclosed in the following U.S. Pat. Nos.: 3,301,746 which issued Jan. 31, 1967, to Lawrence H. Sanford and James B. Sisson; 3,974,025 which issued Aug. 10, 1976, to Peter G. Ayers; 3,994,771 which issued Nov. 30, 1976, to George Morgan, Jr. and Thomas F. Rich; 4,191,609 which issued Mar. 4, 1980, to Paul D. Trokhan; and 4,637,859 which issued Jan. 20, 1987, to Paul D. Trokhan. Each of these papers is characterized by a pattern of dense areas: areas more dense than their respective remainders, such dense areas resulting from being compacted during papermaking as by the crossover knuckles of imprinting carrier fabrics. Other high bulk, soft tissue papers are disclosed in U.S. Pat. No. 4,300,981 which issued Nov. 17, 1981, to Jerry E. Carstens; and U.S. Pat. No. 4,440,597 which issued Apr. 3, 1984, to Edward R. Wells and Thomas A. Hensler. Additionally, achieving high bulk tissue paper through the avoidance of overall compaction prior to final drying is disclosed in U.S. Pat. No. 3,821,068 which issued Jun. 28, 1974, to D. L. Shaw; and avoidance of overall compaction in combination with the use of debonders and elastomeric bonders in the papermak-

ing furnish is disclosed in U.S. Pat. No. 3,812,000 which issued May 21, 1974, to J. L. Salvucci, Jr.

Chemical debonders such as those contemplated by Salvucci, referred to above, and their operative theory are disclosed in such representative U.S. Pat. Nos. as 3,755,220 which issued Aug. 28, 1973, to Friemark et al.; 3,844,880 which issued Oct. 29, 1974, to Meisel et al.; and 4,158,594 which issued Jan. 19, 1979, to Becker et al.

10 Tissue paper has also been treated with cationic surfactants, as well as noncationic surfactants to enhance softness. See, for example, U.S. Pat. No. 4,959,125 which issued Sep. 25, 1990, to Spendel; and U.S. Pat. No. 4,940,513 which issued Jul. 10, 1990, to Spendel, 15 that disclose processes for enhancing the softness of tissue paper by treating it with noncationic, preferably nonionic, surfactants.

It has been found that the softness of tissue paper, in particular, high bulk pattern densified tissue papers, can 20 be improved by treatment with various agents such as vegetable, animal or synthetic oils, and especially polysiloxane materials typically referred to as silicone oils. See, for example, U.S. Pat. No. 5,059,282 which issued Oct. 22, 1991, to Ampulski et al. The Ampulski patent 25 discloses a process for adding a polysiloxane compound to a wet tissue web (preferably at a fiber consistency of between about 20% and about 35%). These polysiloxane compounds impart a silky, soft feeling to the tissue paper. However, addition of the polysiloxane to the 30 tissue web before the web is dried and creped, in accordance with the process disclosed in U.S. Pat. No. '282, can result in interference with the coating on the Yankee dryer and also cause skip crepe and a loss in sheet control. Importantly, these problems are eliminated by 35 the process of the present invention wherein the polysiloxane is added to the tissue sheet after the sheet leaves the Yankee dryer.

U.S. Pat. No. 5,246,546 which issued Sep. 21, 1993 to Ampulski, and incorporated herein by reference discloses an improved process for making soft tissue paper by the application of expensive functional polydimethylpolysiloxane compounds to a dry tissue paper web. Unfortunately, functional polydimethylpolysiloxane compounds are quite expensive, and it is of great economic importance to apply only the minimal quantity required to achieve the desired softness benefit. Surprisingly, Applicant has found that when the functional polydimethylpolysiloxane compounds are first diluted with a miscible, nonvolatile inexpensive solvent such as a nonfunctional polysiloxane compound or a mineral oil, equivalent softness benefits can be obtained with a fraction of the costly functional polydimethylpolysiloxane compounds. It is believed that the addition of the nonfunctional polysiloxane allows the active functional polydimethylpolysiloxane compounds to spread more uniformly on the tissue sheet at lower concentration levels. Importantly, the silicone blends described in the present invention offer substantial cost savings over the higher concentration functional polydimethylpolysiloxane formulations disclosed in U.S. Pat. No. '546.

Additionally, a well known mechanical method of increasing tensile strength of paper made from cellulosic pulp is by mechanically refining the pulp prior to papermaking. In general, greater refining results in greater tensile strength. However, consistent with the foregoing discussion of tissue tensile strength and softness, increased mechanical refining of cellulosic pulp negatively impacts tissue paper softness, all other as-

pects of the papermaking furnish and process being unchanged. However, through the use of the present invention, tensile strength can be increased without negatively impacting softness; or, alternatively, softness can be improved without negatively impacting tensile strength.

It is an object of this invention to provide a process for preparing tissue paper which has an enhanced tactile sense of softness.

It is another object of this invention to provide a process for preparing tissue paper which has a silky, flannel-like feel.

It is another object of this invention to provide a process for preparing tissue paper which has increased tactile softness at a particular level of tensile strength relative to tissue paper which has been softened by conventional techniques.

It is another object to provide a process for preparing a soft tissue paper by applying a functional-polysiloxane compound to a dry tissue web from a thin film.

It is a further object to provide a process for softening tissue paper that only requires very low levels of expensive functional-polysiloxanes compounds.

These and other objects are obtained using the present invention, as will be seen from the following disclosure.

#### SUMMARY OF THE INVENTION

The present invention encompasses a process for making soft tissue paper. This process includes the steps of providing a dry tissue paper web and then applying a sufficient amount of a polysiloxane softener compound to the dry web. More specifically, the softener application process includes the steps of:

- a) providing a dry tissue paper web;
- b) mixing a functional-polysiloxane compound with a suitable nonvolatile diluent to form a functional-polysiloxane containing solution;
- c) mixing the functional-polysiloxane containing solution with a volatile solvent and a suitable surfactant emulsifier to form a functional-polysiloxane containing emulsion;
- d) applying the functional-polysiloxane containing emulsion to a heated transfer surface;
- e) evaporating at least a portion of the volatile solvent from the heated transfer surface to form a film containing the functional polysiloxane compound and the nonvolatile diluent, and
- f) transferring the film from the heated transfer surface to at least one outwardly-facing surface of the tissue web by contacting said outwardly-facing web surface with the heated transfer surface, thereby transferring a sufficient amount of the functional polysiloxane compound such that from about 0.004% to about 0.75% of said functional-polysiloxane compound, based on the dry fiber weight of the tissue web, is retained by the tissue web, and wherein the weight ratio of the functional-polysiloxane compound to the nonvolatile diluent retained by the tissue web ranges from 19:1 to 1:19.

If the volatile solvent in step c) is water then, preferably, the hot web is dried to a moisture level below its equilibrium moisture content (at standard conditions) before being contacted with the polysiloxane film, however this process is also applicable to tissue paper at its

equilibrium moisture as well, if most of the water is evaporated from the transfer surface.

The resulting tissue paper preferably has a basis weight of from about 10 to about 65 g/m<sup>2</sup> and a fiber density of less than about 0.6 g/cc.

As mentioned above, the functional-polysiloxane is applied to the web preferably, after the web has been dried and creped. By adding the polysiloxane to the web after drying and creping, there is no interference with the glue on the Yankee dryer, which can cause skip crepe and/or loss in sheet control. Preferably, the polysiloxane compound is applied to a hot, creped web after it leaves the doctor blade and before it is wound on the parent roll.

Surprisingly, it has been found that significant tissue softening benefits can be achieved by low levels of functional-polysiloxanes when the functional-polysiloxane is blended with a suitable nonvolatile diluent, emulsified with a suitable emulsifier, diluted with a volatile solvent such as water, and applied to a heated transfer surface which evaporates the volatile solvent and then transfers the functional-polysiloxane solution to a hot web before the converting operation. Another advantage of the process disclosed herein, is that the amount of residual volatile solvent transferred to the paper web (e.g., water) is sufficiently low that it does not degrade other product properties.

In addition, the quantity of polysiloxane used is low enough to be economical. It is believed that blending the nonvolatile solvent with the functional-polysiloxane compound allows the functional-polysiloxane compound to spread more uniformly on the tissue sheet at lower concentration levels. Also, tissue paper treated with low levels of polysiloxane retain a high level of wettability, an important feature for a tissue product.

A wide variety of such silicone compounds are known in the art. Specific suitable silicone compositions include, without limitations, polydimethyl siloxanes; mixtures of polydimethyl siloxanes and alkylene oxide-modified polydimethyl siloxanes; organomodified poly-siloxanes; mixtures of cyclic- and non-cyclic-modified dimethyl siloxane; and the like. Number average molecular weights are generally about 10,000 or greater. Also suitable are aqueous mixtures of tetraethoxy silane, dimethyl diethoxy silane, and ethylene oxide/dimethyl siloxane copolymer. Copolymer blends of functional polydimethylpolysiloxane compounds are also suitable, such as mixtures of tetraethoxy silane, dimethyl diethoxy silane, and ethylene oxide-dimethyl siloxane copolymer.

Preferred functional-polysiloxanes for use in the process of the present invention include an amino-functional polydimethylpolysiloxane wherein less than about 10 mole percent of the side chains on the polymer contain an amino-functional group. Because molecular weights of polysiloxanes can be difficult to ascertain, the viscosity of a polysiloxane is used herein as an objectively ascertainable indicia of molecular weight. Accordingly, for example, about 2% substitution has been found to be very effective for polysiloxanes having a viscosity of about one-hundred-twenty-five (125) centistokes; and viscosities of about five-million (5,000,000) centistokes or more are effective with or without substitution. In addition to such substitution with amino-functional groups, effective substitution may be made with carboxyl, hydroxyl, ether, polyether, aldehyde, ketone, amide, ester, and thiol groups. Of these effective substituent groups, the family of groups comprising amino,

carboxyl, hydroxyl, ether and polyether groups are more preferred than the others; and amino-functional groups are most preferred.

Exemplary commercially available functional-polysiloxanes include DOW 8075 which is available from Dow Corning; and Silwet 720 and Ucarsil EPS which are available from Union Carbide.

Suitable nonvolatile diluents include nonfunctional polysiloxane compounds, preferably nonfunctional polydimethyl siloxanes and mineral oils. Examples of nonfunctional polydimethyl siloxanes include SF96-50, SF96-100, SF96-350, SF96-500 all available from General Electric Company, Silicones Division, Waterford, N.Y. Examples of suitable mineral oils include refined aliphatic hydrocarbon solvents, such as PD-23 and PD-25, available from Sonneborn Division, Witco Chemical Corporation, New York, N.Y. Other suitable organic oils include alkanes of approximately C10 and higher, aromatic solvents, halogenated solvents, high molecular weight alcohols, (e.g., lauryl alcohol), higher ketones (e.g., methyl isobutyl ketone), and ethers.

The process for preparing tissue paper treated with a functional-polysiloxane compound in accordance with the present invention may further comprise the step of adding an effective amount of a surfactant to enhance the tactile perceivable surface smoothness of the tissue paper and/or to at least partially offset any reduction of wettability of the tissue paper which would otherwise result from the incorporation of the polysiloxane. The effective amount of surfactant is such that, preferably, from about 0.01 to about 2 percent on a dry fiber weight of the tissue paper; and, more preferably, from about 0.05 to about 1.0 percent is retained by the tissue paper. Also, preferably, the surfactant is noncationic; and is substantially nonmigratory in situ after the tissue paper has been manufactured in order to substantially obviate post-manufacturing changes in the tissue paper's properties which might otherwise result from the inclusion of surfactant. This may be achieved, for instance, through the use of surfactants having melt temperatures greater than the temperatures commonly encountered during storage, shipping, merchandising, and use of tissue paper product embodiments of the invention: for example, melt temperatures of about 50° C. or higher.

Also, the process for preparing tissue paper in accordance with the present invention may further comprise the step of adding an effective amount of a binder material such as starch to at least partially offset any reduction of tensile strength and/or increase in linting propensity which would otherwise result from the incorporation of the polysiloxane and, if present, surfactant material. The effective amount of binder material is such that, preferably, from about 0.01 to about 2 percent on a dry fiber weight basis of the tissue paper, is retained by the tissue paper.

All percentages, ratios and proportions herein are by weight, unless otherwise specified.

#### BRIEF DESCRIPTION OF THE INVENTION

FIG. 1 is a schematic representation illustrating a preferred embodiment of the process of the present invention of adding functional-polysiloxane containing blends to a tissue web.

The present invention is described in more detail below.

#### DETAILED DESCRIPTION OF THE INVENTION

Briefly, the present invention provides tissue paper having a silky, flannel-like feel, and enhanced tactile perceivable softness through the addition of a functional-polysiloxane containing blends to a dry tissue web. The functional-polysiloxane compound is first blended with suitable nonvolatile diluents such as nonfunctional polydimethyl siloxanes and/or organic oils. Preferably, the tissue web is dried to a moisture content below its equilibrium moisture content before the functional-polysiloxane containing material is applied to the web. This process may also include the addition of an effective amount of surfactant material and/or a binder material such as starch to the wet web. Generally speaking, surfactant may be included to enhance tactile perceivable, physiological surface smoothness and/or to assure sufficient wettability for the intended purposes of the tissue paper (e.g., as toilet tissue); and a binder material such as starch may be included to at least partially offset any reduction of tissue paper tensile strength and/or exacerbation of linting propensity which would otherwise be precipitated by the addition of the polysiloxane and, if used, the surfactant.

Surprisingly, it has been found that very low levels of polysiloxane provide a significant tissue softening effect when applied to dry tissue webs in accordance with the present invention. Importantly, it has been found that the levels of functional-polysiloxane used to soften the tissue paper are low enough that the tissue paper retains high wettability. Furthermore, because the tissue web is preferably overdried and at an elevated temperature when the polysiloxane compound is applied, any water added by the polysiloxane solution does not need to be removed. This eliminates the need to further dry the tissue, which might be required if the polysiloxane was added to a tissue web at its equilibrium moisture content.

As used herein, functional polysiloxane compound refers to polysiloxane compounds which have one or more of the following radical groups substituted for one or more alkyl radicals, these include amino, carboxyl, hydroxyl, ether, polyether, aldehyde, ketone, amide, ester, thiol and/or other functionalities including alkyl and alkenyl analogues of such functionalities. For example, an amino functional alkyl group could be an amino-functional or an aminoalkyl-functional polysiloxane. If the amino-functional group replaces a methyl radical on a polydimethylpolysiloxane, it could be referred to as an amino-functional polydimethylpolysiloxane. The exemplary listing of these functional polysiloxanes is not meant to thereby exclude others not specifically listed.

As used herein a nonfunctional-polysiloxane compound refers to polysiloxane compounds wherein the alkyl radicals are not substituted by a functional group.

As used herein a mineral oil refers to a petroleum distillate solvent which has had virtually all aromatic and other unsaturated hydrocarbons removed. It is also known as a liquid paraffin. It is preferably a liquid in which the functional polysiloxane is soluble.

As used herein, nonvolatile miscible diluent refers to a material that is miscible with the functional polysiloxane compound and which has a sufficiently low vapor pressure that essentially most or a large fraction of the quantity applied to the paper does not evaporate and thus it stays with the paper through the processing conditions. Exemplary materials include non-functional

polysiloxane compounds, purified or mixtures of high molecular weight alkanes (approximately greater than decane), mineral oils, and petrolatum. The exemplary listing of these nonvolatile miscible diluents is not meant to thereby exclude others not specifically listed.

As used herein, suitable surfactant emulsifier refers to a surfactant or combination having suitable hydrophilic/lyophilic balance to be able to emulsify the diluted functional polysiloxane mixture. The surfactant should be able to form a sufficiently stable emulsion that the diluted functional polydimethylsiloxane mixture can be applied through the process. Exemplary materials include combinations of sorbitan monolaurates, sorbitan monopalmitates, sorbitan monostearates, polyoxyethylene sorbitan monolaurates, polyoxyethylene sorbitan monopalmitates, polyoxyethylene sorbitan monostearates. The exemplary listing of these emulsifiers is not meant to thereby exclude others not specifically listed.

As used herein, hot tissue web refers to a tissue web which is at an elevated temperature that is higher than room temperature. Preferably the elevated temperature of the web is at least 43° C., and more preferably at least 65° C.

The moisture content of a tissue web is related to the temperature of the web and the relative humidity of the environment in which the web is placed. As used herein, the term "overdried tissue web" refers to a tissue web that is dried to a moisture content below its equilibrium moisture content at standard test conditions of 23° C. and 50% relative humidity. The equilibrium moisture content of a tissue web placed in standard testing conditions of 23° C. and 50% relative humidity is approximately 7%. The tissue web in the present invention can be overdried by raising it to a elevated temperature through use of conventional drying means such as a Yankee dryer. Preferably, an overdried tissue web will have a moisture content of less than 7%, more preferably from about 0 to about 6%, and most preferably, a moisture content of from about 0 to about 3%, by weight.

Paper exposed to the normal environment typically has an equilibrium moisture content in the range of 5 to 8%. When paper is dried and creped the moisture content in the sheet is generally less than 3%. After manufacturing, the paper absorbs water from the atmosphere. In the preferred process of the present invention, advantage is taken of the low moisture content in the paper as it leaves the doctor blade. By applying a polysiloxane solution on the paper while it is overdried, any residual water that is added to the paper is less than what would normally be taken up from the atmosphere. Thus, no further drying is required, and no tensile loss is observed other than that which would normally occur if the paper were absorbing moisture from the air.

The present invention is applicable to tissue paper in general, including but not limited to conventionally felt-pressed tissue paper; pattern densifted tissue paper such as exemplified by Sanford-Sisson and its progeny; and high bulk, uncompacted tissue paper such as exemplified by Salvucci. The tissue paper may be of a homogenous or multilayered construction; and tissue paper products made therefrom may be of a single-ply or multi-ply construction. The tissue paper preferably has a basis weight of between 10 g/m<sup>2</sup> and about 65 g/m<sup>2</sup>, and density of about 0.60 g/cc or less. Preferably, basis weight will be below about 35 g/m<sup>2</sup> or less; and density will be about 0.30 g/cc or less. Most preferably, density will be between 0.04 g/cc and about 0.20 g/cc.

Conventionally pressed tissue paper and methods for making such paper are known in the art. Such paper is typically made by depositing papermaking furnish on a foraminous forming wire. This forming wire is often referred to in the art as a Fourdrinier wire. Once the furnish is deposited on the forming wire, it is referred to as a web. The web is dewatered by pressing the web and drying at elevated temperature. The particular techniques and typical equipment for making webs according to the process just described are well known to those skilled in the art. In a typical process, a low consistency pulp furnish is provided in a pressurized headbox. The headbox has an opening for delivering a thin deposit of pulp furnish onto the Fourdrinier wire to form a wet web. The web is then typically dewatered to a fiber consistency of between about 7% and about 25% (total web weight basis) by vacuum dewatering and further dried by pressing operations wherein the web is subjected to pressure developed by opposing mechanical members, for example, cylindrical rolls. The dewatered web is then further pressed and dried by a stream drum apparatus known in the art as a Yankee dryer. Pressure can be developed at the Yankee dryer by mechanical means such as an opposing cylindrical drum pressing against the web. Multiple Yankee dryer drums may be employed, whereby additional pressing is optionally incurred between the drums. The tissue paper structures which are formed are referred to hereinafter as conventional, pressed, tissue paper structures. Such sheets are considered to be compacted since the web is subjected to substantial overall mechanical compressional forces while the fibers are moist and are then dried while in a compressed state.

Pattern densifted tissue paper is characterized by having a relatively high bulk field of relatively low fiber density and an array of densifted zones of relatively high fiber density. The high bulk field is alternatively characterized as a field of pillow regions. The densifted zones are alternatively referred to as knuckle regions. The densifted zones may be discretely spaced within the high bulk field or may be interconnected, either fully or partially, within the high bulk field. Preferred processes for making pattern densifted tissue webs are disclosed in U.S. Pat. No. 3,301,746, issued to Sanford and Sisson on Jan. 31, 1967, U.S. Pat. No. 3,974,025, issued to Peter G. Ayers on Aug. 10, 1976, and U.S. Pat. No. 4,191,609, issued to Paul D. Trokhan on Mar. 4, 1980, and U.S. Pat. No. 4,637,859, issued to Paul D. Trokhan on Jan. 20, 1987; all of which are incorporated herein by reference.

In general, pattern densifted webs are preferably prepared by depositing a papermaking furnish on a foraminous forming wire such as a Fourdrinier wire to form a wet web and then juxtaposing the web against an array of supports. The web is pressed against the array of supports, thereby resulting in densifted zones in the web at the locations geographically corresponding to the points of contact between the array of supports and the wet web. The remainder of the web not compressed during this operation is referred to as the high bulk field. This high bulk field can be further dedensified by application of fluid pressure, such as with a vacuum type device or a blow-through dryer, or by mechanically pressing the web against the array of supports. The web is dewatered, and optionally predried, in such a manner so as to substantially avoid compression of the high bulk field. This is preferably accomplished by fluid pressure, such as with a vacuum type device or blow-through

dryer, or alternately by mechanically pressing the web against an array of supports wherein the high bulk field is not compressed. The operations of dewatering, optional predrying and formation of the densifted zones may be integrated or partially integrated to reduce the total number of processing steps performed. Subsequent to formation of the densifted zones, dewatering, and optional predrying, the web is dried to completion, preferably still avoiding mechanical pressing. Preferably, from about 8% to about 55% of the tissue paper surface comprises densifted knuckles having a relative density of at least 125% of the density of the high bulk field.

The array of supports is preferably an imprinting carrier fabric having a patterned displacement of knuckles which operate as the array of supports which facilitate the formation of the densifted zones upon application of pressure. The pattern of knuckles constitutes the array of supports previously referred to. Imprinting carrier fabrics are disclosed in U.S. Pat. No. 3,301,746, Sanford and Sisson, issued Jan. 31, 1967, U.S. Pat. No. 3,821,068, Salvucci, Jr. et al., issued May 21, 1974, U.S. Pat. No. 3,974,025, Ayers, issued Aug. 10, 1976, U.S. Pat. No. 3,573,164, Friedberg et al., issued Mar. 30, 1971, U.S. Pat. No. 3,473,576, Amneus, issued Oct. 21, 1969, U.S. Pat. No. 4,239,065, Trokhan, issued Dec. 16, 1980, and U.S. Pat. No. 4,528,239, Trokhan, issued Jul. 9, 1985, all of which are incorporated herein by reference.

Preferably, the furnish is first formed into a wet web on a foraminous forming carrier, such as a Fourdrinier wire. The web is dewatered and transferred to an imprinting fabric. The furnish may alternately be initially deposited on a foraminous supporting carrier which also operates as an imprinting fabric. Once formed, the wet web is dewatered and, preferably, thermally predried to a selected fiber consistency of between about 40% and about 80%. Dewatering is preferably performed with suction boxes or other vacuum devices or with blow-through dryers. The knuckle imprint of the imprinting fabric is impressed in the web as discussed above, prior to drying the web to completion. One method for accomplishing this is through application of mechanical pressure. This can be done, for example, by pressing a nip roll which supports the imprinting fabric against the face of a drying drum, such as a Yankee dryer, wherein the web is disposed between the nip roll and drying drum. Also, preferably, the web is molded against the imprinting fabric prior to completion of drying by application of fluid pressure with a vacuum device such as a suction box, or with a blow-through dryer. Fluid pressure may be applied to induce impression of densifted zones during initial dewatering, in a separate, subsequent process stage, or a combination thereof.

Uncompacted, nonpattern-densified tissue paper structures are described in U.S. Pat. No. 3,812,000 issued to Joseph L. Salvucci, Jr. and Peter N. Yiannos on May 21, 1974, and U.S. Pat. No. 4,208,459, issued to Henry E. Becker, Albert L. McConnell, and Richard Schutte on Jun. 17, 1980, both of which are incorporated herein by reference. In general, uncompacted, nonpattern-densified tissue paper structures are prepared by depositing a papermaking furnish on a foraminous forming wire such as a Fourdrinier wire to form a wet web, draining the web and removing additional water without mechanical compression until the web has a fiber consistency of at least 80%, and creping the

web. Water is removed from the web by vacuum dewatering and thermal drying. The resulting structure is a soft but weak high bulk sheet of relatively uncompacted fibers. Bonding material is preferably applied to portions of the web prior to creping.

Compacted non-pattern-densified tissue structures are commonly known in the art as conventional tissue structures. In general, compacted, non-pattern-densified tissue paper structures are prepared by depositing a papermaking furnish on a foraminous wire such as a Fourdrinier wire to form a wet web, draining the web and removing additional water with the aid of a uniform mechanical compaction (pressing) until the web has a consistency of 25-50%, transferring the web to a thermal dryer such as a Yankee and creping the web. Overall, water is removed from the web by vacuum, mechanical pressing and thermal means. The resulting structure is strong and generally of singular density, but very low in bulk, absorbency and in softness.

The papermaking fibers utilized for the present invention will normally include fibers derived from wood pulp. Other cellulosic fibrous pulp fibers, such as cotton linters, bagasse, etc., can be utilized and are intended to be within the scope of this invention. Synthetic fibers, such as rayon, polyethylene and polypropylene fibers, may also be utilized in combination with natural cellulosic fibers. One exemplary polyethylene fiber which may be utilized is Pulpex TM, available from Hercules, Inc. (Wilmington, Del.).

Applicable wood pulps include chemical pulps, such as Kraft, sulfite, and sulfate pulps, as well as mechanical pulps including, for example, groundwood, thermomechanical pulp and chemically modified thermomechanical pulp. Chemical pulps, however, are preferred since they impart a superior tactile sense of softness to tissue sheets made therefrom. Pulps derived from both deciduous trees (hereinafter, also referred to as "hardwood") and coniferous trees (hereinafter, also referred to as "softwood") may be utilized. Also applicable to the present invention are fibers derived from recycled paper, which may contain any or all of the above categories as well as other nonfibrous materials such as fillers and adhesives used to facilitate the original papermaking.

In addition to papermaking fibers, the papermaking furnish used to make tissue paper structures may have other components or materials added thereto as may be or later become known in the art. The types of additives desirable will be dependent upon the particular end use of the tissue sheet contemplated. For example, in products such as toilet paper, paper towels, facial tissues and other similar products, high wet strength is a desirable attribute. Thus, it is often desirable to add to the papermaking furnish chemical substances known in the art as "wet strength" resins.

A general dissertation on the types of wet strength resins utilized in the paper art can be found in TAPPI monograph series No. 29, Wet Strength in Paper and Paperboard, Technical Association of the Pulp and Paper Industry (New York, 1965). The most useful wet strength resins have generally been cationic in character. Polyamide-epichlorohydrin resins are cationic permanent wet strength resins which have been found to be of particular utility. Suitable types of such resins are described in U.S. Pat. Nos. 3,700,623, issued on Oct. 24, 1972, and 3,772,076, issued on Nov. 13, 1973, both issued to Keim and both being hereby incorporated by reference. One commercial source of a useful poly-

mide-epichlorohydrin resins is Hercules, Inc. of Wilmington, Del., which markets such resin under the mark Kymene TM 557H.

Polyacrylamide resins have also been found to be of utility as permanent wet strength resins. These resins are described in U.S. Pat. Nos. 3,556,932, issued on Jan. 19, 1971, to Coscia, et al. and 3,556,933, issued on Jan. 19, 1971, to Williams et al., both patents being incorporated herein by reference. One commercial source of polyacrylamide resins is American Cyanamid Co. of Stamford, Conn., which markets one such resin under the mark Parez TM 631 NC.

Still other water-soluble cationic resins finding utility in this invention are urea formaldehyde and melamine formaldehyde resins. The more common functional groups of these polyfunctional resins are nitrogen containing groups such as amino groups and methylol groups attached to nitrogen. Polyethylenimine type resins may also find utility in the present invention. In addition, starch-based temporary wet strength resins such as Caldas 10 (manufactured by Japan Carlit) and CoBond 1000 (manufactured by National Starch and Chemical Company) may be used in the present invention. It is to be understood that the addition of chemical compounds such as the wet strength and temporary wet strength resins discussed above to the pulp furnish is optional and is not necessary for the practice of the present development.

Types of polysiloxane materials which are suitable for use in the present invention include polymeric, oligomeric, copolymeric, and other multiple-monomeric siloxane materials. As used herein, the term polysiloxane and silicone are used interchangeably. They shall include all of such polymeric, oligomeric, copolymeric and other multiple-monomeric siloxane materials. Additionally, the polysiloxane can be either a straight chain, a branched chain or have a cyclic structure.

Preferred polysiloxane materials include those having monomeric siloxane units of the following structure:



(1)

wherein, R<sub>1</sub> and R<sub>2</sub> for each siloxane monomeric unit can independently be any alkyl, aryl, alkenyl, alkaryl, aralkyl, cycloalkyl, halogenated hydrocarbon, or other radical. Any of such radicals can be substituted or unsubstituted. R<sub>1</sub> and R<sub>2</sub> radicals of any particular monomeric unit may differ from the corresponding functionalities of the next adjoining monomeric unit. Additionally, the radicals can be either a straight chain, a branched chain, or have a cyclic structure. The radicals R<sub>1</sub> and R<sub>2</sub> can, additionally and independently, be other silicone functionalities such as, but not limited to siloxanes, polysiloxanes, and polysilanes. The radicals R<sub>1</sub> and R<sub>2</sub> can also contain any of a variety of organic functionalities including, for example, alcohol, carboxylic acid, and amine functionalities.

The degree of substitution and the type of substituent have been found to affect the relative degree of soft, silky feeling and hydrophilicity imparted to the tissue paper structure. In general, the degree of soft, silky feeling imparted by the polysiloxane increases as the hydrophilicity of the substituted polysiloxane decreases.

Aminofunctional polysiloxanes are especially preferred in the present invention.

Preferred polysiloxanes include straight chain organopolysiloxane materials of the following general formula:



wherein each R<sub>1</sub>-R<sub>9</sub> radical can independently be any C<sub>1</sub>-C<sub>10</sub> unsubstituted alkyl or aryl radical, and R<sub>10</sub> is any substituted C<sub>1</sub>-C<sub>10</sub> alkyl or aryl radical. Preferably each R<sub>1</sub>-R<sub>9</sub> radical is independently any C<sub>1</sub>-C<sub>4</sub> unsubstituted alkyl group. Those skilled in the art will recognize that technically there is no difference whether, for example, R<sub>9</sub> or R<sub>10</sub> is the substituted radical. Preferably the mole ratio of b to (a+b) is between 0 and about 20%, more preferably between 0 and about 10%, and most preferably between about 1% and about 5%.

In one particularly preferred embodiment, R<sub>1</sub>-R<sub>9</sub> are methyl groups and R<sub>10</sub> is a substituted or unsubstituted alkyl, aryl, or alkenyl group. Such material shall be generally described herein as polydimethylsiloxane which has a particular functionality as may be appropriate in that particular case. Exemplary polydimethylsiloxanes include, for example, polydimethylsiloxane, polydimethylsiloxane having an alkyl hydrocarbon R<sub>10</sub> radical and polydimethylsiloxane having one or more amino, carboxyl, hydroxyl, ether, polyether, aldehyde, ketone, amide, ester, thiol and/or other R<sub>10</sub> functionalities including alkyl and alkenyl analogues of such functionalities. For example, an amino functional alkyl group as R<sub>10</sub> could be an amino-functional or an aminoalkylfunctional polydimethylsiloxane. The exemplary listing of these functional-polydimethylsiloxanes is not meant to thereby exclude others not specifically listed.

Viscosity of polysiloxanes useful for this invention may vary as widely as the viscosity of polysiloxanes in general vary, so long as the polysiloxane is flowable or can be made to be flowable for application to the tissue paper. This includes, but is not limited to, viscosity as low as about 25 centistokes to about 20,000,000 centistokes or even higher. High viscosity polysiloxanes which themselves are resistant to flowing can be effectively deposited upon the tissue paper webs by such methods as, for example, emulsifying the polysiloxane in surfactant or providing the polysiloxane in solution with the aid of a solvent, such as hexane, listed for exemplary purposes only. Particular methods for applying polysiloxanes to tissue paper webs are discussed in more detail below.

Parenthetically, while not wishing to be bound by a theory of operation, it is believed that the tactile-benefit efficacy of the polysiloxane is directly related to its average molecular weight; and that viscosity is directly related to molecular weight. Accordingly, due to the relative difficulty of directly determining molecular weights of polysiloxanes as compared to determining their viscosities, viscosity is used herein as the apparent operative parameter with respect to imparting enhanced tactile response to tissue paper: i.e., softness, silkiness, and flannel-like.

References disclosing polysiloxanes include U.S. Pat. No. 2,826,551, issued Mar. 11, 1958, to Geen; U.S. Pat. No. 3,964,500, issued Jun. 22, 1976, to Drakoff; U.S. Pat. No. 4,364,837, issued Dec. 21, 1982, to Pader; and British Patent 849,433, published Sep. 28, 1960, to Woolston. Also, *Silicon Compounds*, pp. 181-217, distributed by Petrarch Systems, Inc., 1984, contains an extensive listing and description of polysiloxanes in general.

While not wishing to be bound by theory it is believed that the softness benefit of functional polydimethyl siloxane compounds is primarily that of improving surface lubricity as opposed to changing the bulk properties such as flexibility. The unique feature of functional polydimethyl siloxane compounds is their ability to work at very low levels. However it is believed, that the benefit is not just concentration dependent, but it is a surface coverage dependent. That is to say, it is believed that a minimum degree of surface coverage is required for softness to be improved. The thickness of the coverage can be very thin, on the order of perhaps several monolayers, as opposed to hundreds or greater. Once an optimal degree of surface coverage has been obtained the softness improvement appears to level off. Application of more functional polydimethyl siloxane compound does not significantly continue to improve softness.

Since, functional polydimethyl siloxane compounds are quite expensive it is of great economic importance to apply only the minimal quantity required to achieve the required softness benefit. Applying more only leads to increased cost and no further improved softness benefit. It has been surprising to learn that some processes are more efficient at improving softness than others. That is, significantly less functional polydimethyl siloxane compound is required to reach the maximum softness benefit. Other processes require ten to one hundred or more times the quantity to reach essentially the same softness benefit. In the most efficient process, high volumes of a very dilute functional polydimethyl siloxane emulsion are sprayed on the sheet surface. Due to the large volumes of water applied to the paper the paper needs to be dried with for example thermal energy to remove the excess water. In an attempt to not have to dry the sheet after the functional polydimethyl siloxane emulsion has been applied a process was devised in which the functional polydimethyl siloxane was sprayed on an over dried sheet. The applied moisture was only enough to bring the sheet to its equilibrium moisture content. In another process the polydimethyl siloxane emulsion was sprayed on a heated transfer roll, where the water was evaporated leaving a thin film of functional polydimethyl siloxane compound which was subsequently transferred to the paper surface. While this method of application is preferred, since it does not require further drying of the sheet and it does not interfere with Yankee coatings and result in a loss in sheet control, this process requires the use of more functional polydimethylpolysiloxane to deliver the desired softness benefit. While waterless volatile solvents would work from a theoretical aspect, the practical limitations on these materials from a safety and environmental standpoint does not make them feasible to use in a paper making system. Diluting the functional polydimethyl siloxane with large quantities of nonvolatile solvents would also work to deliver the desired end softness benefit. However the paper product would then retain

the solvent and it could impart a potentially unpleasant consumer attribute, such as an oily or greasy feel.

A surprising observation was made when the following mixture was formulated and applied to an overdried paper substrate. The functional polydimethylpolysiloxane compound was first diluted with a miscible solvent such as a low weight mineral oil e.g., Witco PD-23 available from Witco Corporation, New York, N.Y. The solution was then emulsified and diluted with water. The emulsion was sprayed on a heated transfer roll where a portion of the water evaporated leaving a thin film of the functional polydimethylpolysiloxane/mineral oil solution. The thin film was then transferred to the paper substrate. It was surprising to find that the softness benefit could be delivered with a fraction of the functional polydimethyl siloxane compound delivered from the nonvolatile containing emulsion as compared to that where the functional polydimethyl siloxane compound was applied to the overdried sheet without the nonvolatile solvent. The nonvolatile solvent had no appreciable softness improvement benefit on its own. That is, in the absence of the functional polydimethyl siloxane compound, the softness was not significantly enhanced with only the application of the nonvolatile solvent. The total quantity of nonvolatile solvent applied was not sufficient to be noticeable to the consumer. It is believed that the addition of the miscible nonvolatile solvent allows the active functional polydimethyl silicone compound to spread either on the heated transfer surface and or in the sheet to a thin level, thus delivering the optimum degree of surface coverage that is required for softness. Even though the quantity is less, the degree of surface coverage remains adequate since it is dispersed in the nonvolatile diluents.

Suitable nonvolatile diluents include nonfunctional polydimethyl siloxanes and organic oils. Examples of nonfunctional polydimethyl siloxanes include SF96-50, SF96-100, SF96-350, SF96-500 all available from General Electric Company, Silicones Division, Waterford, N.Y. Examples of suitable organic oils include refined aliphatic hydrocarbon solvents, such as PD-23 and PD-25, available from Sonneborn Division, Witco Chemical Corporation, New York, N.Y., mineral oils, alkanes of approximately C10 and higher, aromatic solvents, halogenated solvents, high molecular weight alcohols, (e.g., lauryl alcohol), higher ketones (e.g., methyl isobutyl ketone), and ethers.

The useful properties of the nonvolatile diluent include the ability to form a miscible solution with the functional polydimethyl siloxane. The viscosity of the nonfunctional polydimethyl siloxane diluents can be in the range of about 25 to about 1000 centistokes as measured at 77° F. The viscosity of the organic diluent materials can be in the range of about 25 to 1000 SUS as measured at 100° F. (ASTM D2161-63T). The material should not interfere with the spreading of the functional polydimethyl siloxane. The flash point should be above approximately 150° F. (ASTM D92).

Preferred materials that have been found to work include the nonfunctional polydimethyl siloxane SF96-350 and the organic materials PD-23 and PD-25.

A useful way to prepare the softening material for application to the sheet is to combine and mix the functional polydimethyl siloxane with the nonvolatile diluent. The solution is then emulsified with a suitable emulsifier known to those skilled in the art. The emulsified functional polydimethyl nonvolatile diluent mixture is

then diluted with water and applied to the paper substrate.

Although less preferred, it may also be possible to mix the nonvolatile diluent with an already emulsified functional polydimethyl siloxane then diluting the combined mixture with water and applying the material to a paper substrate. Another method of preparing the softener system for application is to mix an emulsified functional polydimethyl siloxane with an emulsified nonvolatile diluent.

The most preferred method is to first combine and mix the functional polydimethyl siloxane with the nonvolatile diluent. The solution is then emulsified with a suitable emulsifier known to those skilled in the art. The emulsified functional polydimethyl nonvolatile diluent mixture is then diluted with water and applied to the paper substrate.

Useful combination ratios of functional polydimethyl siloxane to nonvolatile diluent are, as those skilled in the art will realize, dictated by economics at one end and wanting to deliver the useful benefit at the other end. One would obviously want to dilute an expensive material with as much low cost material as possible to minimize cost. However, there will be a limit above which further dilution will result in a loss in softness response by the consumer. While weight ratios of 95 parts functional polydimethyl siloxane to 5 parts nonvolatile diluent to 5 parts functional polydimethyl siloxane to 95 parts nonvolatile diluent fit the broadest scope, a more preferred range 75 parts functional polydimethyl siloxane to 25 parts nonvolatile diluent to 10 parts functional polydimethyl siloxane to 90 parts nonvolatile diluent. An even more preferred range is 50 parts functional polydimethyl siloxane to 50 parts nonvolatile diluent to 15 parts functional polydimethyl siloxane to 85 parts nonvolatile diluent.

The functional-polysiloxane/nonvolatile diluent solution is applied after the tissue web has been dried and creped, and preferably is still at an elevated temperature. It has been found that addition of a polysiloxane compound to the tissue web before the web is dried and creped can result in interference with the coating on the dryer (i.e., glue coating on Yankee dryer), and also cause skip crepe and a loss in sheet control. These problems are eliminated by the process of the present invention wherein the polysiloxane compounds are applied to the web after the web has been dried and creped. Preferably, the polysiloxane compounds are applied to the dried and creped tissue web before the web is wound onto the parent roll.

It has also been found that application of the polysiloxane followed by calendering of the tissue web further enhances the softness of the tissue product. Without being bound by theory, it is believed that the calender aids in distribution of the polysiloxane by working the sheet and moving the polysiloxane around on the fiber surfaces. Thus, in a preferred embodiment of the present invention the polysiloxane compound is applied to a hot, overdried tissue web after the web has been creped, but before the web passes through the calender rolls.

The functional-polysiloxane is preferably applied to the hot transfer surface from an aqueous solution, emulsion, or suspension. The functional polysiloxane is most preferably applied in a solution containing a suitable, nonvolatile diluent, in which the functional polysiloxane dissolves or with which the polysiloxane is miscible: for example, a non-functional polysiloxane or mineral

oil. The diluted polysiloxane may be mixed with water or, more preferably, emulsified in water with a suitable surfactant emulsifier. Emulsified polysiloxane is preferable for ease of application, since a simple mixture of polysiloxane in water must be agitated to inhibit separation into water and polysiloxane phases.

The functional-polysiloxane/nonvolatile diluent solution should be applied uniformly to the transfer surface for subsequent uniform transfer to the tissue paper web

10 so that substantially the entire sheet benefits from the tactile effect of the polysiloxane. Applying the functional-polysiloxane/nonvolatile diluent solution to the tissue paper web in continuous and patterned distributions are both within the scope of the invention and meet the 15 above criteria. Likewise, the functional-polysiloxane/-nonvolatile diluent solution can be added to either side of the tissue web singularly, or to both sides.

Methods of uniformly applying the functional-polysiloxane/nonvolatile diluent solution to the hot transfer surface include spraying and gravure printing. Spraying has been found to be economical, and susceptible to accurate control over quantity and distribution of the functional-polysiloxane, so it is most preferred. Preferably, an aqueous mixture containing an emulsified 25 functional-polysiloxane blended with a nonvolatile diluent is applied from the transfer surface onto the dried, creped tissue web after the Yankee dryer and before the parent roll. FIG. 1 illustrates a preferred method of applying the functional-polysiloxane containing emulsion to the tissue web. Referring to FIG. 1, a wet tissue web 1 is on carrier fabric 14 past turning roll 2 and transferred to Yankee dryer 5 by the action of pressure roll 3 while carrier fabric 14 travels past turning roll 16. The paper web is adhesively secured to the cylindrical 30 surface of Yankee dryer 5 by adhesive applied by spray applicator 4. Drying is completed by steam-heated Yankee dryer 5 and by hot air which is heated and circulated through drying hood 6 by means not shown. The web is then dry creped from the Yankee dryer 5 by doctor blade 7, after which it is designated creped paper sheet 15. An aqueous mixture containing an emulsified 35 functional-polysiloxane compound and nonvolatile diluent is sprayed onto an upper heated transfer surface designated as upper calender roll 10 and/or a lower heated transfer surface designated as lower calender roll 11, by spray applicators 8 and 9 depending on whether the functional-polysiloxane compound is to be applied to both sides of the tissue web or just to one side. The paper sheet 15 then contacts heated transfer

40 surfaces 10 and 11 after a portion of the solvent has been evaporated. The treated web then travels over a circumferential portion of reel 12, and thence is wound onto parent roll 13. Equipment suitable for spraying polysiloxane-containing liquids onto hot transfer surfaces include external mix, air atomizing nozzles, such as the 2 mm nozzle available from V.I.B. Systems, Inc., Tucker, Ga. Equipment suitable for printing polysiloxane-containing liquids onto hot transfer surfaces include rotogravure printers.

45 50 55 60 65 60 While not wishing to be bound by theory or to otherwise limit the present invention, the following description of typical process conditions encountered during the papermaking operation and their impact on the process described in this invention is provided. The Yankee dryer raises the temperature of the tissue sheet and removes the moisture. The steam pressure in the Yankee is on the order of 110 PSI (750 kPa). This pressure is sufficient to increase the temperature of the cyl-

inder to about 173° C. The temperature of the paper on the cylinder is raised as the water in the sheet is removed. The temperature of the sheet as it leaves the doctor blade can be in excess of 120° C. The sheet travels through space to the calender and the reel and loses some of this heat. The temperature of the paper wound in the reel is measured to be on the order of 65° C. Eventually the sheet of paper cools to room temperature. This can take anywhere from hours to days depending on the size of the paper roll. As the paper cools it also absorbs moisture from the atmosphere. As previously mentioned, the moisture content in the sheet is related to the sheet temperature and the relative humidity of the environment in which the paper is placed. For example the equilibrium moisture content of a sheet placed in standard testing conditions of 23° C. and 50% RH is approximately 7%. Increasing the moisture content of the sheet above 7% can have a deleterious effect on the tensile strength of the paper. For example, a moisture increase to 9% can cause the tensile strength of the paper to decrease by as much as 15%.

One very surprising attribute of functional-polysiloxane softeners is their ability to improve softness at very low levels on the surface of the paper. The polysiloxane softener, however needs to be fairly uniformly distributed on the paper surface in order for the consumer to recognize the improved softness. From a process standpoint, there was previously no satisfactory method of uniformly applying low quantities of a polysiloxane compound to a paper web traveling at a high rate of speed. Belt speeds of 700 to 1000 meters/minute (25 to 40 miles/hour) are typical in modern high speed paper machines. Webs traveling at these rates of speed generally have an air boundary layer on their surface. One method for applying low quantities of liquids is to use a spray system and adjust the air and/or liquid pressures. For example, one could go to low flow rates by using high air pressures. This generally produces extremely small particles. It is difficult to impart sufficient momentum into these small particles so they can penetrate the air boundary layer traveling on the surface of the fast moving paper web. Moreover, if one increases the particle size of the spray fluid so it can penetrate the air boundary layer at low flow rates the surface coverage becomes nonuniform.

One commonly used method for applying low levels of an active material is to first dilute the material with a solvent or a diluent. The spray systems can then be adjusted to deliver larger particle sizes at high flow rates. The larger particles can penetrate the air boundary layer. However one is now faced with the problem of having to remove the solvent or diluent from the paper. Generally volatile organic solvents are not used in papermaking, since they can be fire or environmental hazards. Water can be used as a diluent, for the polysiloxane, if the polysiloxane is first emulsified with a suitable surfactant system. While water does not pose the same process risks as an organic solvent, water can degrade the product, causing a loss in crepe and/or tensile strength. Further the water needs to be removed from the paper.

One solution to the water problem is to apply a dilute polysiloxane solution to the paper while it is overdried. The water added to the paper by this method is usually less than the paper would normally take up from the atmosphere upon cooling to room temperature. Thus, no further drying is required, and no loss in tensile strength occurs from addition of the water. However,

the water solution is capable of penetrating the entire sheet causing the active material to spread to the inside of the sheet rather than staying on the surface of the paper where it is most effective. Further, this process is limited to an overdried sheet, making application to the paper during a converting process (an off paper machine process) difficult without adding an additional drying step to the process. A further limitation to this process is the limited dilution range and application range of the polysiloxane emulsion imposed by the emulsion properties, (i.e., high concentrations tend to have high viscosities, whereas low concentrations increase the amount of water sprayed on the sheet).

The process used in the present invention solves the above described problems by first spraying a dilute emulsified polysiloxane solution onto a hot transfer surface and evaporating the solvent from the polysiloxane solution before transferring it to the dry web. For exemplary purposes, a typical commercially available functional silicone Dow 8075 marketed by the Dow Corning Corporation. This material is an amino-functional polysiloxane. This material is diluted to a 25% solution with Witco PD-23 a mineral oil marketed by Witco Chemical Corporation. This mixture is then emulsified in water. The mixed emulsion is diluted with water to less than about 20% concentration, by weight, before being applied to the heated transfer surface. More preferably, silicone emulsions used in the present invention are first diluted with water to less than about 15% concentration by weight before being applied to the transfer surface.

Exemplary materials suitable for the heated transfer surfaces include metal, e.g., steel, stainless steel, and chrome and rubber. When the diluted polysiloxane emulsion was sprayed on the hot transfer surface, in this case a steel calender roll, it was most surprising to discover that little or no water was transferred to the paper web by this process. In fact, under one set of process conditions, it was expected that the sheet moisture content would increase from a base of 4% to 5% after spraying. However, it was found that the moisture content did not increase at all, while the silicone content in the web did increase to its expected concentration. It was a further surprise to find that an attempt to increase the sheet moisture by 3.5% (i.e., raising the sheet moisture from 4 to 7.5%) only resulted in a moisture increase of 0.7%, that is the measured moisture content was only 4.7%.

This is most surprising since the roll temperature is on the order of 80° C. (20° C. below the boiling point of water) and the time between the point of application and point of transfer is on the order of 0.1 sec. It was surprising to discover that greater than 50% of the water had evaporated from the roll under these conditions, leaving behind a thin film of polysiloxane emulsion. This thin film was calculated to be on the order of 0.25 microns thick (1 micron=10<sup>-6</sup> meters). The films of the present invention are preferably less than about 10 microns in thickness, and more preferably, less than about one micron in thickness.

By thin film is meant any thin coating, haze or mist on the transfer surface. This thin film can be microscopically continuous, discrete, or patterned, but should be macroscopically uniform.

In the process of the present invention it is preferred that at least about 50%, more preferably at least about 80%, of the water is evaporated from the dilute polysiloxane emulsion applied to the heated transfer surface

before transferring it to the dry tissue web. This leaves a film, with a calculated thickness of about 0.075 microns thick. Most preferably greater than about 95% of the water is evaporated from the emulsion on the heated transfer surface, leaving a calculated film thickness of about 0.05 microns for transfer to the paper web.

The heat on the transfer surface can also cause a lowering of the polysiloxane viscosity, thus increasing its ability to spread into a thin film on the transfer surface. This film is then transferred to the paper web surface by contacting the web with the transfer surface. Surprisingly, it has been found that the polysiloxane transfer efficiency to the web is quite high. Efficiencies on the order of 40 to 80% are typical, based on the flow out of the spray nozzles to the transfer surface and the quantity measured on the paper web. Moreover, this process is not limited to overdried paper. Depending on the amount of water removed from the spray mixture by the hot transfer surface, the process described herein is capable of delivering polysiloxane softeners to equilibrated dry paper as well. However application to a hot overdried web is preferred, to insure that any residual water in the film does not interfere with any paper properties.

An additional benefit in applying the polysiloxane solution to a hot overdried web is that the decreased viscosity of the solution aids in insuring that the solution is uniformly applied across the surface of the web. (It is believed that the low viscosity solution is more mobile).

It has been found, surprisingly, that low levels of polysiloxane applied to hot, overdried tissue paper webs can provide a softened, silky, flannel-like, nongreasy tactile sense of feel to the tissue paper without the aid of additional materials such as oils or lotions. Importantly, these benefits can be obtained for many of the embodiments of the present invention in combination with high wettability within the ranges desirable for toilet paper application. Preferably, tissue paper treated with functional-polysiloxane compounds in accordance with the present invention comprises about 0.75% or less of the functional-polysiloxane. It is an unexpected benefit of this invention that tissue paper treated with about 0.75% or less polysiloxane can have imparted thereto substantial softness and silkiness benefits by such a low level of polysiloxane. In general, tissue paper having less than about 0.75% polysiloxane, preferably less than about 0.5%, can provide substantial increases in softness and silkiness and flannel-like quality yet remain sufficiently wettable for use as toilet paper without requiring the addition of surfactant to offset any negative impact on wettability which results from the polysiloxane.

The minimum level of functional-polysiloxane to be retained by the tissue paper is at least an effective level for imparting a tactile difference in softness or silkiness or flannel-like quality to the paper. The minimum effective level may vary depending upon the particular type of sheet, the method of application, the particular type of polysiloxane, and whether the polysiloxane is supplemented by starch, surfactant, or other additives or treatments. Without limiting the range of applicable polysiloxane retention by the tissue paper, preferably at least about 0.004%, more preferably at least about 0.01%, and most preferably at least about 0.05% polysiloxane is retained by the tissue paper.

Preferably, a sufficient amount of a functional-polysiloxane to impart a tactile sense of softness is disposed uniformly on both surfaces of the tissue paper:

i.e., disposed on the outwardly facing surfaces of the surface-level fibers. When polysiloxane is applied to one surface of the tissue paper, some of it will, generally, at least partially penetrate to the tissue paper interior. However, preferably, the polysiloxane is applied to both sides of the tissue paper to ensure that both surfaces have imparted thereto the benefits of the polysiloxane.

In addition to treating tissue paper with polysiloxane as described above, it has been found desirable to also treat such tissue paper with surfactant material. This is in addition to any surfactant material that may be present as an emulsifying agent for the polysiloxane.

Tissue paper having in excess of about 0.3% polysiloxane is preferably treated with surfactant when contemplated for uses wherein high wettability is desired. Most preferably, a noncationic surfactant is applied to the hot, overdried tissue paper web, in order to obtain an additional softness benefit, on a constant tensile basis, as previously discussed. The amount of surfactant required to increase hydrophilicity to a desired level will depend upon the type and level of polysiloxane and the type of surfactant. However, as a general guideline, between about 0.01% and about 2% surfactant retained by the tissue paper, preferably between about 0.05% and about 1.0%, is believed to be sufficient to provide sufficiently high wettability for most applications, including toilet paper, for polysiloxane levels of about 0.75% or less.

Surfactants which are preferred for use in the present invention are noncationic; and, more preferably, are nonionic. However, cationic surfactants may be used. Noncationic surfactants include anionic, nonionic, amphoteric, and zwitterionic surfactants. Preferably, as stated hereinbefore, the surfactant is substantially non-migratory in situ after the tissue paper has been manufactured in order to substantially obviate post-manufacturing changes in the tissue paper's properties which might otherwise result from the inclusion of surfactant. This may be achieved, for instance, through the use of surfactants having melt temperatures greater than the temperatures commonly encountered during storage, shipping, merchandising, and use of tissue paper product embodiments of the invention: for example, melt temperatures of about 50°C. or higher. Also, the surfactant is preferably water-soluble when applied to the wet web.

The level of noncationic surfactant applied to tissue paper webs to provide the aforementioned softness/tensile benefit ranges from the minimum effective level needed for imparting such benefit, on a constant tensile basis for the end product, to about two (2) percent: preferably between about 0.01% and about 1% noncationic surfactant retained by the web; more preferably, between about 0.05% and about 1.0%; and, most preferably, between about 0.05% and about 0.3%.

The surfactants preferably have alkyl chains with eight or more carbon atoms. Exemplary anionic surfactants are linear alkyl sulfonates, and alkylbenzene sulfonates. Exemplary nonionic surfactants are alkylglycosides including alkylglycoside esters such as Crodesta TM SL-40 which is available from Croda, Inc. (New York, N.Y.); alkylglycoside ethers as described in U.S. Pat. No. 4,011,389, issued to W. K. Langdon, et al. on Mar. 8, 1977; linear primary alcohol ethoxylates such as Noedol ® 25-12 available from Shell Chemical Co. (Houston, Tex.); and alkylpolyethoxylated esters such as Pegosperse TM 200 ML available from Glyco Chem-

icals, Inc. (Greenwich, Conn.). Alkylpolyglycosides are particularly preferred for use in the present invention. The above listings of exemplary surfactants are intended to be merely exemplary in nature, and are not meant to limit the scope of the invention.

The surfactant, in addition to any emulsifying surfactant that may be present on the polysiloxane, may be applied by the same methods and apparatuses used to apply polysiloxanes. These methods include spraying and gravure printing. Other methods include application to a forming wire or fabric prior to contact with the web. Any surfactant other than polysiloxane emulsifying surfactant material, is hereinafter referred to as "surfactant," and any surfactant present as the emulsifying component of emulsified polysiloxane is hereinafter referred to as "emulsifying agent".

The surfactant may be applied to the tissue paper simultaneously with, after, or before the polysiloxane, in a typical process, the surfactant is applied to an overdried web simultaneously with the polysiloxane, that is, the surfactant is included in the dilute polysiloxane solution applied to the heated transfer surface.

As stated hereinbefore, it is also desirable to treat polysiloxane containing tissue paper with a relatively low level of a binder for lint control and/or to increase tensile strength. As used herein the term "binder" refers to the various wet and dry strength additives known in the art. The binder may be applied to the tissue paper simultaneously with, after or before the polysiloxane and the surfactant, if used. In some instances, binders are added to the overdried tissue webs simultaneously with the polysiloxane (i.e., the binder is included in the dilute polysiloxane solution applied to the heated transfer surface).

Polyamide-epichlorohydrin resins have been found to be the preferred binder for use in the present invention. Preferably, the tissue paper fibers are treated with an aqueous solution of a polyamide-epichlorohydrin resin before the sheet is formed. In addition to reducing linting of the finished tissue paper product, low levels of polyamide-epichlorohydrin resin also imparts an improvement in the wet strength of the tissue paper.

Starch-based resins have been found to be useful as temporary wet strength agents in the present invention. In general, suitable starch for practicing the present invention is characterized by water solubility, and hydrophilicity. Exemplary starch materials include corn starch and potato starch, albeit it is not intended to thereby limit the scope of suitable starch materials; and waxy corn starch that is known industrially as amioica starch is particularly preferred. Amioica starch differs from common corn starch in that it is entirely amylopectin, whereas common corn starch contains both amylopectin and amylose. Various unique characteristics of amioica starch are further described in "Amioica-The Starch From Waxy Corn", H. H. Schopmeyer, Food Industries, December 1945, pp. 106-108 (Vol. pp. 1476-1478).

The starch can be in granular or dispersed form albeit granular form is preferred. The starch is preferably sufficiently cooked to induce swelling of the granules. More preferably, the starch granules are swollen, as by cooking, to a point just prior to dispersion of the starch granule. Such highly swollen starch granules shall be referred to as being "fully cooked." The conditions for dispersion in general can vary depending upon the size of the starch granules, the degree of crystallinity of the granules, and the amount of amylose present. Fully

cooked amioica starch, for example, can be prepared by heating an aqueous slurry of about 4% consistency of starch granules at about 190° F. (about 88° C.) for between about 30 and about 40 minutes.

Other exemplary starch materials which may be used include modified cationic starches such as those modified to have nitrogen containing groups such as amino groups and methylol groups attached to nitrogen, available from National Starch and Chemical Company, (Bridgewater, N.J.). Such modified starch materials have heretofore been used primarily as a pulp furnish additive to increase wet and/or dry strength. However, when applied in accordance with this invention by application to an overdried tissue paper web they may have reduced effect on wet strength relative to wet-end addition of the same modified starch materials. Considering that such modified starch materials are more expensive than unmodified starches, the latter have generally been preferred.

Starch is preferably applied to tissue paper webs in an aqueous solution. Methods of application include, the same previously described with reference to application of polysiloxane: preferably by spraying; and, less preferably, by printing. The starch may be applied to the tissue paper web simultaneously with, prior to, or subsequent to the addition of polysiloxane and/or surfactant.

At least an effective amount of a binder, preferably starch, to provide lint control and concomitant strength increase upon drying relative to a non-binder treated but otherwise identical sheet is preferably applied to the sheet. Preferably, between about 0.01% and about 2.0% of a binder is retained in the dried sheet, calculated on a dry fiber weight basis; and, more preferably, between about 0.1% and about 1.0% of a binder material, preferably starch-based, is retained. As mentioned above, polyamide-epichlorohydrin resins are preferred when permanent wet strength is desired (e.g., in facial tissue products).

Analysis of the amounts of treatment chemicals herein retained on tissue paper webs can be performed by any method accepted in the applicable art. For example, the level of polysiloxane retained by the tissue paper can be determined by solvent extraction of the polysiloxane with an organic solvent followed by atomic absorption spectroscopy to determine the level of silicon in the extract; the level of nonionic surfactants, such as alkylglycosides, can be determined by extraction in an organic solvent followed by gas chromatography to determine the level of surfactant in the extract; the level of anionic surfactants, such as linear alkyl sulfonates, can be determined by water extraction followed by colorimetry analysis of the extract; the level of starch can be determined by amylase digestion of the starch to glucose followed by colorimetry analysis to determine glucose level. These methods are exemplary, and are not meant to exclude other methods which may be useful for determining levels of particular components retained by the tissue paper.

Hydrophilicity of tissue paper refers, in general, to the propensity of the tissue paper to be wetted with water. Hydrophilicity of tissue paper may be somewhat quantified by determining the period of time required for dry tissue paper to become completely wetted with water. This period of time is referred to as "wetting time." In order to provide a consistent and repeatable test for wetting time, the following procedure may be used for wetting time determinations: first, a conditioned sample unit sheet (the environmental conditions

for testing of paper samples are  $23^{\circ}\pm 1^{\circ}$  C. and  $50\pm 2\%$  RH. as specified in TAPPI Method T 402), approximately  $4\frac{1}{8}$  inch  $\times$   $4\frac{1}{8}$  inch (about 11.1 cm  $\times$  12 cm) of tissue paper structure is provided; second, the sheet is folded into four (4) juxtaposed quarters, and then crumpled into a ball approximately 0.75 inches (about 1.9 cm) to about 1 inch (about 2.5 cm) in diameter; third, the balled sheet is placed on the surface of a body of distilled water at  $23^{\circ}\pm 1^{\circ}$  C. and a timer is simultaneously started; fourth, the timer is stopped and read when wetting of the balled sheet is completed. Complete wetting is observed visually.

The preferred hydrophilicity of tissue paper depends upon its intended end use. It is desirable for tissue paper used in a variety of applications, e.g., toilet paper, to completely wet in a relatively short period of time to prevent clogging once the toilet is flushed. Preferably, wetting time is 2 minutes or less. More preferably, wetting time is 30 seconds or less. Most preferably, wetting time is 10 seconds or less.

Hydrophilicity characters of tissue paper embodiments of the present invention may, of course, be determined immediately after manufacture. However, substantial increases in hydrophobicity may occur during the first two weeks after the tissue paper is made: i.e., after the paper has aged two (2) weeks following its manufacture. Thus, the above stated wetting times are preferably measured at the end of such two week period. Accordingly, wetting times measured at the end of a two week aging period at room temperature are referred to as "two week wetting times."

The density of tissue paper, as that term is used herein, is the average density calculated as the basis weight of that paper divided by the caliper, with the appropriate unit conversions incorporated therein. Caliper of the tissue paper, as used herein, is the thickness of the paper when subjected to a compressive load of 95 g/in<sup>2</sup> (15.5 g/cm<sup>2</sup>).

#### EXAMPLE I

The purpose of this example is to illustrate one method that can be used to make soft tissue paper sheets treated with a functional polysiloxane in accordance with the present invention.

A pilot scale Fourdrinier papermaking machine is used in the practice of the present invention. The paper machine has a layered headbox having a top chamber, a center chamber, and a bottom chamber. Where applicable as indicated in the following examples, the procedure described below also applies to such later examples. Briefly, a first fibrous slurry comprised primarily of short papermaking fibers is pumped through the top and bottom headbox chambers and, simultaneously, a second fibrous slurry comprised primarily of long papermaking fibers is pumped through the center headbox chamber and delivered in superposed relation onto the Fourdrinier wire to form thereon a three-layer embryonic web. The first slurry has a fiber consistency of about 0.11% and its fibrous content is Eucalyptus Hardwood Kraft. The second slurry has a fiber consistency of about 0.15% and its fibrous content is Northern Softwood Kraft. Dewatering occurs through the Fourdrinier wire and is assisted by a deflector and vacuum boxes. The Fourdrinier wire is 84M supplied by Albany International (Appleton, Wis.). The embryonic wet web is transferred from the Fourdrinier wire, at a fiber consistency of about 22% at the point of transfer, to a carrier fabric having a 5-shed weave, 44 machine-direction

and 33 cross-machine-direction monofilaments per inch, respectively. The warp configuration is 4 over and 1 under. The shute configuration is 1 over and 4 under. The warp pick sequence delta is 2. The web is carried on the carrier fabric past the vacuum dewatering box, through the blow-through predryers after which the web is transferred onto a Yankee dryer. The fiber consistency is about 27% after the vacuum dewatering box and, by the action of the predryers, about 65% prior to transfer onto the Yankee dryer; creping adhesive comprising a 0.25% aqueous solution of polyvinyl alcohol is spray applied by applicators; the fiber consistency is increased to an estimated 99% before dry creping the web with a doctor blade. The doctor blade has a bevel angle of about 24 degrees and is positioned with respect to the Yankee dryer to provide an impact angle of about 83 degrees; the Yankee dryer is operated at about 350° F. (177° C.); the Yankee dryer is operated at about 800 fpm (feet per minute) (about 244 meters per minute). The heated calender rolls are sprayed with a polysiloxane emulsion, further described below, using a 2 mm spray nozzle. The web is then passed between the two heated calender rolls. The two calender rolls are biased together at roll weight and operated at surface speeds of 660 fpm (about 201 meters per minute).

The spray solution is made by diluting 25 parts of Dow Corning 8075 (an amino-functional polydimethylpolysiloxane marketed by Dow Corning Corp.) with 75 parts Witco PD-23 (a petroleum distillate solvent available from Witco Chemical Corporation, New York, N.Y.). The mixture is emulsified and then diluted to 3% by weight with water. The aqueous diluted polysiloxane solution is then sprayed onto the heated lower steel calender roll. The volumetric flow rate of the aqueous solution through the nozzle is about 2 gal/hr per cross-direction ft (about 25 liters/hr-meter). Greater than about 95% of the water is evaporated from the calender rolls leaving the diluted functional polysiloxane. The dry web, which has a moisture content of about 1%, contacts the hot calender rolls. The diluted functional polysiloxane compound and the nonfunctional compound are transferred to the dry web by direct pressure transfer. The transfer efficiency of the polysiloxane applied to the web, in general, is about 45%.

The resulting tissue paper has a basis weight of 30 g/m<sup>2</sup>, a density of 0.10 g/cc, and contains 0.0250% by weight, of the amino-functional polydimethylpolysiloxane compound, 0.075% by weight, of Witco PD-23 and has an unequilibrated initial moisture content of 1.2%.

#### EXAMPLE II

The purpose of this example is to illustrate one method that can be used to make soft tissue paper sheets wherein the tissue paper is treated with polysiloxane, surfactant and starch.

A 3-layer paper sheet is produced in accordance with the hereinbefore described process of Example I. The tissue web is, in addition to being treated with a diluted functional polysiloxane compound as described above, also treated with Crodesta TM SL-40 (an alkyl glycoside polyester nonionic surfactant marketed by Croda Inc.) and with a fully cooked amioica starch prepared as described in the specification. The surfactant and starch are applied simultaneously with the emulsified polysiloxane composition as part of the aqueous solution sprayed through the papermachine spray nozzle. Concentration of the Crodesta TM SL-40 nonionic surfactant in the aqueous solution is adjusted so that the level

of surfactant retained is about 0.10%, based upon the weight of the dry fibers. Similarly, concentration of the starch in the aqueous solution is adjusted so that the level of amioca starch retained is about 0.2%, based upon the weight of the dry fibers.

The treating mixture is sprayed onto an upper and a lower heated transfer roll. The water is evaporated from the rolls and the diluted functional polysiloxane, surfactant, and binder is transferred to both sides of the tissue web. The volumetric flow rate through the upper and lower spray nozzle onto the heated rolls is about 1 gal/hr per cross-direction ft. The combined flow rate through both nozzles is 2 gal/hr per cross-direction ft.

The resulting tissue paper has a basis weight of 30 g/m<sup>2</sup>, a density of 0.10 g/cc, and contains 0.0250% by weight of the amino-functional polydimethylsiloxane, 0.075% by weight, of Witco PD-23, 0.1% by weight of Crodesta TM SL-40 nonionic surfactant and 0.2% by weight of the cooked amioca starch. Importantly, the resulting tissue paper has a silky flannel-like feel, enhanced tactile softness and has higher wettability and lower propensity for lint than tissue paper treated only with the polysiloxane composition.

### EXAMPLE III

The purpose of this example is to illustrate one method that can be used to make soft tissue paper sheets wherein the tissue paper is treated in accordance with the present invention and converted into a two ply product.

A 2-layer paper sheet is produced in accordance with the hereinbefore described process of Example I with the following exceptions. The volumetric flow rate through the nozzle is approximately 1.05 gal/hr per cross-direction foot (about 13.3 liters/hr-meter). The film thickness after 95% of the water is evaporated is calculated to about 0.035 microns. The resulting single ply tissue paper has a basis weight of 16 g/m<sup>2</sup>.

Following papermaking, two sheets of treated paper are combined together with the treated surfaces facing outward.

The resulting two-ply tissue paper product has a basis weight of 32 g/m<sup>2</sup>, a density of 0.10 g/cc, and contains 0.025% by weight, of the amino-functional polydimethylsiloxane and 0.075% Witco PD-23.

Importantly, the resulting tissue paper has a silky, flannel-like feel, and enhanced tactile softness.

### EXAMPLE IV

The purpose of this example is to illustrate a method using conventional drying and layered paper making techniques to make soft, absorbent and lint resistant multi-ply facial tissue paper treated with a functional polysiloxane in accordance with the present invention and a permanent wet strength resin and a dry strength resin.

A pilot scale Fourdrinier paper making machine is used in the practice of the present invention. First, the chemical softener composition is prepared according to the procedure in Example I.

Second, a 3% by weight aqueous slurry of NSK is made up in a conventional re-pulper. The NSK slurry is refined gently and a 2% solution of the permanent wet strength resin (i.e. Kymene TM 557H marketed by Hercules Incorporated of Wilmington, Del.) is added to the NSK stock pipe at a rate of 0.3% by weight of the dry fibers. The adsorption of the permanent wet strength resin onto NSK fibers is enhanced by an in-line mixer. A

1% solution of the dry strength resin (i.e. CMC from Hercules Incorporated of Wilmington, DE) is added to the NSK stock before the fan pump at a rate of 0.05% by weight of the dry fibers. The NSK slurry is diluted to about 0.2% consistency at the fan pump.

Third, a 3% by weight aqueous slurry of Eucalyptus fibers is made up in a conventional re-pulper. A 2% solution of the permanent wet strength resin (i.e. Kymene TM 557H) is added to the Eucalyptus stock pipe at a rate of 0.1% by weight of the dry fibers, followed by addition of a 1% solution of CMC at a rate of 0.025% by weight of the dry fibers.

The individually treated furnish streams (stream 1-100% NSK/stream 2=100% Eucalyptus) are kept separate through the headbox and deposited onto a Fourdrinier wire to form a two layer embryonic web containing equal portions of NSK and Eucalyptus. De-watering occurs through the Fourdrinier wire and is assisted by a deflector and vacuum boxes. The Fourdrinier wire is of a 5-shed, satin weave configuration having 110 machine-direction and 95 cross-machine-direction monofilaments per inch, respectively. The embryonic wet web is transferred from the Fourdrinier wire, at a fiber consistency of about 8% at the point of trans-

fer, to a pickup felt (Superfine Duracomb, Style Y-31675-1, Albany International, Albany, N.Y.). Further de-watering is accomplished by vacuum assisted drainage until the web has a fiber consistency of about 35%. The web is then adhered to the surface of a Yankee dryer. The fiber consistency is increased to an estimated 96% before dry creping the web with a doctor blade. The doctor blade has a bevel angle of about 25 degrees and is positioned with respect to the Yankee dryer to provide an impact angle of about 81 degrees; the Yankee dryer is operated at about 800 fpm (feet per minute) (about 244 meters per minute). The emulsified softener solution is sprayed on the lower calender stack as described in the process of Example I with the following exceptions. The volumetric flow rate through the nozzle is approximately 1.05 gal/hr cross-direction foot (about 13.3 liters/hr-meter). The film thickness after 95% of the water is evaporated is calculated to about 0.035 microns. The dry web is formed into a roll at a speed of 650 fpm (200 meters per minutes). The resulting single ply tissue paper has a basis weight of 16 g/m<sup>2</sup>.

Following papermaking, two sheets of treated paper are combined together with the treated surfaces facing outward.

The resulting two-ply tissue paper product has a basis weight of 32 g/m<sup>2</sup>, a density of 0.10 g/cc, and contains about 0.2% of the permanent wet strength resin, about 0.0375% of the dry strength resin, and about 0.025% by weight, of the amino-functional polydimethylsiloxane and 0.075% Witco PD-23.

Importantly, the resulting tissue paper has a silky, flannel-like feel, and enhanced tactile softness.

What is claimed is:

1. A process for applying low levels of a functional-polysiloxane compound and a mineral oil to a dry tissue paper web, said process comprising the steps of:
  - a) providing a dry tissue paper web;
  - b) mixing a functional-polysiloxane compound with a suitable mineral oil to form a functional-polysiloxane containing solution;
  - c) mixing said functional-polysiloxane containing solution with water and a suitable surfactant emulsifier to form a functional-polysiloxane containing emulsion.

- d) applying said functional-polysiloxane containing emulsion to a heated transfer surface;
- e) evaporating at least a portion of the water from said heated transfer surface to form a film containing said functional polysiloxane and said mineral oil, and
- f) transferring said film from said heated transfer surface to at least one outwardly-facing surface of said tissue web by contacting said outwardly-facing web surface with said heated transfer surface, thereby transferring a sufficient amount of said functional polysiloxane compound such that from about 0.004% to about 0.75% of said functional polysiloxane compound, based on the dry fiber weight of said tissue web, is retained by said tissue web, and wherein the weight ratio of the functional-polysiloxane compound to the mineral oil retained by the tissue web ranges from 19:1 to 1:19.

2. The process of claim 1 wherein from about 0.01% to about 0.3% of said functional-polysiloxane is retained by said web.

3. The process of claim 1 wherein the mineral oil in step (b) is a petroleum distillate solvent.

4. The process of claim 1 wherein the weight ratio of the functional polysiloxane compound to the mineral oil retained by the tissue web ranges from 1:9 to 3:1.

5. The process of claim 1 wherein said functional-polysiloxane is a polydimethyl polysiloxane having a hydrogen bonding functional group selected from the groups consisting of amino, carboxyl, hydroxyl, ether, polyether, aldehyde, ketone, amide, ester and thiol groups, said hydrogen bonding functional group being present in a molar percentage of substitution of about 20% or less.

6. The process of claim 5 wherein said functional-polysiloxane has a molar percentage of substitution of about 10% or less, and a viscosity of about 25 centistokes or more.

7. The process of claim 6 wherein said functional-polysiloxane has a molar percentage of substitution of from about 1.0% to about 5%, and a viscosity of from about 25 centistokes to about 20,000,000 centistokes.

8. The process of claim 7 wherein said molar percentage of substitution is about 2%, and said viscosity is about 125 centistokes.

9. The process of claim 5 wherein said hydrogen bonding functional group is an amino functional group.

10. The process of claim 1 further comprising the step of applying to said web, a sufficient amount of water soluble surfactant such that from about 0.01% to about 2.0% of said surfactant, based on the dry fiber weight of said tissue paper, is retained by said web.

11. The process of claim 10 wherein said surfactant is noncationic.

12. The process of claim 11 wherein said noncationic surfactant is a nonionic surfactant.

13. The process of claim 10 wherein said surfactant has a melting point of at least about 50° C.

14. The process of claim 1 further comprising the step of applying to said web, a sufficient amount of a binder such that from about 0.01% to about 2.0% of said binder, based on the dry fiber weight of said tissue paper, is retained by said web.

15. The process of claim 14 wherein said binder is a permanent wet strength resin.

16. The process of claim 15 wherein said permanent wet strength resin is a polyamide-epichlorohydrin resin.

17. The process of claim 14 wherein said binder is a temporary wet strength resin.

18. The process of claim 17 wherein said temporary wet strength resin is a starch-based resin.

19. The process of claim 10 further comprising the step of applying to said web, a sufficient amount of a binder such that from about 0.01% to about 2.0% of said binder, based on the dry fiber weight of said tissue paper, is retained by said web.

20. The process of claim 19 wherein said surfactant is noncationic, said binder is a polyamide-epichlorohydrin resin, and said mineral oil is a petroleum distillate solvent.

21. The process of claim 20 wherein said heated transfer surface is a calender roll.

22. The product made by the process of claim 1.

23. The product made by the process of claim 21.

\* \* \* \* \*

UNITED STATES PATENT AND TRADEMARK OFFICE  
**CERTIFICATE OF CORRECTION**

PATENT NO. : 5,389,204  
DATED : February 14, 1995  
INVENTOR(S) : Robert Stanley Ampulski

Page 1 of 1

It is certified that error appears in the above-identified patent and that said Letters Patent is hereby corrected as shown below:

Title page,

Under Assignee, please delete "Proctger" and insert therefor -- Procter --.

Column 2,

Line 19, delete "densifted" and insert therefor -- densified --.

Column 3,

Line 12, after feel, delete "," and insert therefor -- . --.

Column 7,

Line 57, delete "densifted" and insert therefor -- densified --.

Column 8,

Lines 34, 36, 38, 40, 43, 51, and 56, delete "densifted" and insert therefor -- densified --.

Column 9,

Lines 4, 7, 11, 17 and 53, delete "densifted" and insert therefor -- densified --.

Signed and Sealed this

Twelfth Day of March, 2002

Attest:

Attesting Officer



JAMES E. ROGAN  
Director of the United States Patent and Trademark Office